

1

3,253,908

STAINLESS STEEL AND METHOD  
Harry Tanczyn, Baltimore, Md., assignor to Armco  
Steel Corporation, a corporation of Ohio  
No Drawing. Filed Nov. 20, 1959, Ser. No. 854,226  
5 Claims. (Cl. 75—124)

This invention relates to the heat-hardenable chromium-nickel-aluminum steels, more particularly the composition of the steel, a method of heat-hardening the same, and the resulting hardened steel itself.

Among the objects of the invention is the provision of a particular chromium-nickel-aluminum stainless steel which is comparatively soft and workable in one condition of heat-treatment and which readily may be hardened for use or service by treatment at temperatures which are not unduly high, to achieve a hard, strong and tough steel, a steel having excellent hardness and strength at room temperatures and at elevated temperatures together with reasonably good ductility and impact strengths, which stainless steel lends itself to hot-working as by forging, rolling and piercing, into a variety of flat, round special shapes for fabrication and heat-treatment to yield a host of articles and products of ultimate use made to the desired specification and tolerances with a minimum loss of metal in treatment.

Other objects of my invention in part will be obvious and in part pointed out in the course of the following specification.

My invention accordingly resides in the combination of elements and relative proportioning of the same, as well as in the various heat-treating steps and the relation of each of the same to one or more of the others, and in the final heat-treated product, all as described herein and particularly set forth in the claims at the end of this specification.

As conducive to a better understanding of certain features of my invention it may be noted at this point that the stainless steels generally are defined as those steels which comprise about 10% to 35% chromium, with or without nickel, and with or without additions of any one or more of a number of ingredients employed for special purposes. These ingredients commonly include small amounts of silicon, copper, cobalt, molybdenum, aluminum, tungsten, vanadium, titanium, columbium, and the like. The carbon and manganese contents usually are low, although for special purposes, these may be substantial.

Many grades of stainless steel are now on the market. Of these it generally is considered that it is the chromium-nickel grades which possess the best working and forming characteristics. These steels readily may be hot-worked and cold-worked. They may be bent, pressed, stamped, punched and machined to form a host of useful articles, products and component parts. And many of the chromium-nickel stainless steels are greatly benefited through the addition of one or more of the strong carbide-forming elements titanium and columbium. Others are benefited through the addition of copper. And in still others through the addition of aluminum.

The chromium-nickel-aluminum stainless steels presently available not only are comparatively soft, ductile and readily workable in one condition of heat-treatment, but they are easily hardened by heat-treatment to give a steel which is of substantial strength. In many applications, however, it is found that these steels suffer in ductility and impact strength and that greater hardness and higher strength at room temperatures and elevated temperatures are desirable.

One of the objects of my invention, therefore, is to provide a particular chromium-nickel-aluminum stainless

2

steel which possesses the many desirable characteristics of the known chromium-nickel-aluminum stainless steels in matters of workability and formability, as well as subsequent hardenability, together with improved hot-working conditions at the steel mill in addition to possessing improved hardness and strength in heat-hardened condition, both at room temperatures and at elevated temperatures, and in addition possesses improved ductility and impact strength.

10 In the practice of my invention I provide a chromium-nickel-aluminum stainless steel of substantial molybdenum and nitrogen contents and a minimum carbon content. The chromium content of my steel amounts to about 9% to 20%, the nickel content from 2.50% to 15 8.00%, manganese up to 8.00%, with manganese inversely proportioned with respect to the nickel content, the aluminum from .70% to 2.50%, the molybdenum content 1.0% to 5.0%, with the sum of the chromium and molybdenum contents 14% to 21%, the nitrogen content from .10% to .40%, and the carbon content not exceeding .12%, with remainder substantially all iron. The proportioning of these several ingredients is in every sense critical. Where the chromium content is less than 9% and the sum of the chromium and molybdenum 20 contents less than 14%, the corrosion resistance characteristics seriously suffer. And where the chromium exceeds 20% and the sum of the chromium and molybdenum contents exceeds 21%, I find that inadequate hardening is achieved. The molybdenum content of the 25 steel is at least 1%, for with less than this both hardness and strength suffer. And with more than 5% it appears that there is a loss of corrosion resistance in certain media. Moreover, no benefit seems to derive from an excess of molybdenum. And it is an expensive addition.

30 35 A nickel content of anything less than 2.50% gives a steel which is objectionably hard in the annealed condition with consequent loss of forming properties. With a nickel content exceeding 8.00% I find that the steel inadequately responds to heat-treatment and fails to 40 develop the desired hardness in the final heat-hardened condition.

45 Manganese, of course, is present, this in amounts up to 2.00% as a maximum. Where desired, however, the nickel content of the steel may be partially replaced by manganese on a 2 for 1 basis, that is, 2% manganese for every 1% of nickel replaced. But I find that there must be an actual nickel content of at least 2.50%, and that the total manganese content, this including the 50 amounts commonly present and the amounts employed for replacing the nickel, shall not exceed 8%. For with an excessive amount of manganese there is a loss of ductility and impact strength in the final heat-hardened condition.

55 55 The aluminum content is critical, too, for with an aluminum content less than .70% inadequate hardening is had and where it exceeds 2.50% the steel suffers a loss of hardenability, does not harden to the full extent.

In my steel the carbon content should not exceed .12% because with a higher carbon content I find a definite 60 loss of corrosion resistance, especially in pickling the steel as with the known nitric acid-hydrofluoric acid pickling solutions commonly used to remove heat-tint from the heat-treating operations referred to hereinafter. Actually, I much prefer that the carbon content shall 65 not exceed 0.08% in order to positively assure freedom from corrosive attack.

Both molybdenum and nitrogen are essential ingredients as noted above. For I find that both lend hardness to the steel in final heat-treated condition. And nitrogen contributes to ductility and impact strength. Where there is employed nitrogen in amount less than .10%, the high ductility and impact strength of my steel is lost. And

where it substantially exceeds .40% the composition balance is adversely affected; the steel is inclined to become objectionably hard in the annealed condition with consequent loss of working and forming properties.

The silicon content of my steel amounts to about 2.00% as a maximum, the phosphorus content a maximum of .050%, and the sulphur content a maximum of .050%.

The steel of my invention therefore essentially consists of chromium in the amount of 9% to 20%, nickel in the amount of 2.50% to 8.00%, manganese a maximum of 8.00% with manganese 8.00% when nickel is 2.5% and 2% maximum where nickel is 8.00%, aluminum in the amount of .70% to 2.00%, molybdenum in amount of 1% to 5%, with the sum of the chromium and molybdenum contents 14% to 21%, nitrogen in the amount of .10% to .40%, carbon .12% maximum, preferably .08% maximum, and more particularly a maximum of .03%, with silicon 2.0% maximum, phosphorus and sulphur each .050% maximum, with the remainder of the steel substantially all iron. The preferred steel of my invention as appears more fully hereinafter analyzes 15.0% to 16.0% chromium, 6.0% to 7.5% nickel, .8% to 1.5% aluminum, 2.0% to 3.0% molybdenum, .10% to .20% nitrogen, carbon .08% maximum, manganese 1.5% maximum, silicon 1.0% maximum, with the remainder substantially all iron.

My steel is melted in accordance with the procedures generally described and claimed in one or more of the U.S. Letters Patent 1,925,182 of September 5, 1933, issued to Alexander L. Feild, and entitled, "Process for the Manufacture of Rustless Iron," Patent 2,455,073, issued November 30, 1948, to Donald L. Loveless and entitled, "Production of Stainless Steel," and Patent 2,621,119 of December 9, 1952, issued to Donald L. Loveless and entitled, "Stainless Steel Melting Process." The required nitrogen content is conveniently introduced in the manner described in the Weitzenkorn U.S. Patent 2,454,020 of November 16, 1948, entitled, "Ferrochrome Process and Product." For the steels of high manganese, nitrogen is introduced in accordance with the method described in U.S. Patent 2,696,433 of December 9, 1954, entitled, "Production of High Nitrogen-Manganese Steel."

The steel, obtained in the form of ingots, is fashioned into blooms and billets and thence converted into plate, sheet, strip, bars, rods, wire and tubes at the mill. I find that it possesses improved hot-working characteristics, this as compared with the prior chromium-nickel-aluminum stainless steels.

The various converted products are annealed at a temperature of 1800° to 2100° F. and either cooled in air or quenched in water, as desired. The time at annealing temperature does not appear to be particularly critical; usually one-half hour at temperature is sufficient. The steel in the annealed condition is substantially fully austenitic, any free-ferrite not exceeding about 10% by volume. The aluminum content of the steel appears to remain in solution even after quenching or cooling. The metal is reasonably soft and ductile. The hardness does not exceed Rockwell B99. It is readily worked and formed as by bending, drawing, spinning. And it is easily machined. Moreover, it may be welded, by known methods such as the electric arc or the gas torch. With fabrication there are had a variety of articles, products and parts for industry and commerce. The steel is readily fashioned into various structural members required for airplanes. It is easily made into bolts, screws and nuts. It is suitably fashioned into valves and valve parts, die blocks and surgical instruments. In the working, forming and fabrication of the steel particular advantage is taken

of its good workability and formability in the annealed condition. These various working, forming and fabricating operations, of course, are usually performed by the customer-fabricator.

Following fabrication the various articles, products and parts are heated at a temperature of about 1400° F. for a sufficient length of time to effect a precipitation of the carbides present in the steel, presumably carbides of chromium. There also may be some precipitation of aluminum compounds. And the steel, upon cooling, as by water-quench, transforms into martensite or a martensite-like constituent with some free-ferrite present. The steel in this condition, for a typical example, has a hardness amounting to some Rockwell C28/29.

The high molybdenum, high nitrogen chromium-nickel-aluminum stainless steel of my invention retains sufficient softness and ductility in the preliminarily hardened condition to permit working as by cold-rolling and drawing, and machining as by turning, cutting, punching, drilling, and the like. Where desired, therefore, one or more of the various working, forming and fabricating operations referred to above may be delayed and practiced on the preliminarily hardened steel rather than upon the annealed metal coming from the mill.

In the further practice of my invention I find that as a result of the preliminary hardening treatment at a temperature of some 1400° F. there is formed on the various stainless steel articles, products and parts a light heat-tint. It is conveniently removed by pickling in an aqueous solution of nitric and hydrofluoric acids. In general, the nitric acid content amounts to about 15% by volume and the hydrofluoric acid about 2%, with remainder water. My steel is possessed of superior corrosion resisting properties; even the thinnest sections, that is, sections on the order of .005" to .010", are reliably pickled without fear of metal loss or penetration through the metal as occasionally encountered in the steels of the prior art. My steel in no way suffers from intergranular attack. This I attribute to the extremely low carbon content, with the consequent formation of a bare minimum of objectionable carbides.

The preliminary hardened chromium-nickel-aluminum stainless steels of high molybdenum and nitrogen contents and low carbon content are now given a final hardening treatment by reheating at a temperature of about 1050° F. for about an hour. While the temperature may range from some 750° to 1100° F. for a time of half an hour at the higher temperature to some 2 hours or more at the lower temperature, I find that a temperature of 1050° F. gives excellent results. With final hardening treatment and cooling in air or water the martensite or martensite-like constituent of the preliminarily hardened steel is fully retained.

In the final hardening treatment, it is my view that there is precipitated an aluminum compound, very likely a compound of nickel and aluminum, which gives rise to the further hardening. It may be that the hardening reaction involves some rearrangement or reordering of the lattice structure of the aluminum compound within the lattice structure of the austenitic matrix. However all that may be, the steel of my invention, as finally hardened by heat-treatment, is hard and strong and yet reasonably ductile and tough. The hardness had amounts to some Rockwell C42 as a minimum.

As specifically illustrative of my invention I have prepared two chromium-nickel-aluminum stainless steels of high molybdenum and nitrogen contents and low carbon content. The chemical analyses of these examples are given in Table I below:

TABLE I.—CHEMICAL ANALYSES OF Cr-Ni-Al STAINLESS STEELS OF HIGH MOYBDENUM AND NITROGEN CONTENTS, AND LOW CARBON CONTENT

| Heat No.  | C    | Mn  | P    | S    | Si  | Cr    | Ni   | Al   | Mo   | N   |
|-----------|------|-----|------|------|-----|-------|------|------|------|-----|
| R440----- | .018 | .56 | .008 | .011 | .51 | 15.03 | 7.37 | 1.04 | 2.53 | .12 |
| R423----- | .063 | .55 | .010 | .007 | .57 | 15.30 | 7.30 | 1.06 | 2.49 | .15 |

The two specific examples of my stainless steel as illustratively set forth above were annealed at a temperature of 1900° for a period of one-half hour and then quenched in water. Following annealing and quenching they were heated at a temperature of 1400° F. for a period of 1½ hrs. and water-quenched, after which they were reheated at 1050° F. for 1½ hrs. and cooled in air. The hardness had in these several samples in the various conditions of annealing, preliminary hardening and final hardening are given in Table II below:

TABLE II.—HARDNESS VALUES OF THE TWO STEELS OF TABLE I IN THE ANNEALED, PRELIMINARILY HARDENED AND FINAL HARDENED CONDITION

| Heat No.  | Annealed<br>(1,900° F.,<br>1/2 hr. W.Q.) | Pre. Hard. (An-<br>nealed plus<br>1,400° F.,<br>90 min. W.Q.) | Final Hard. (Pre-<br>Hard. plus 1,050° F.,<br>1/2 hr. and A.C.) |
|-----------|------------------------------------------|---------------------------------------------------------------|-----------------------------------------------------------------|
| R440----- | Rockwell B99                             | Rockwell C27                                                  | Rockwell C43.                                                   |
| R423----- | Rockwell B94                             | Rockwell C28                                                  | Rockwell C46.                                                   |

The mechanical properties of the two illustrative steels are given below in Table III:

TABLE III.—MECHANICAL PROPERTIES OF THE STEELS OF TABLE I IN THE FINAL HARDENED CONDITION (1,900° F. FOR 1/2 HR. W.Q.+1,400° F. FOR 1/2 HRS. A.C.+1,050° F. FOR 1/2 HRS. A.C.)

| Heat No.  | U.T.S.,<br>p.s.i. | 0.2% Y.S.,<br>p.s.i. | Percent<br>El. in 2" | Percent<br>Red. Area | Izod<br>Impact<br>(Ft./Lbs.) | Rockwell<br>Hardness |
|-----------|-------------------|----------------------|----------------------|----------------------|------------------------------|----------------------|
| R440----- | 200,000           | 187,200              | 16.0                 | 54.0                 | 8-9                          | C43                  |
| R423----- | 221,000           | 198,000              | 12.5                 | 45.7                 | 2-4                          | C47                  |

It will be seen that I provide in my invention a chromium-nickel-aluminum steel in which there are had the various objects hereinbefore set forth, together with many practical advantages. The chromium-nickel-aluminum stainless steel of my invention of high molybdenum and nitrogen contents and low carbon content works well in the mill, is of improved corrosion resistance and readily lends itself to forming and fabrication by well known methods. These include bending, spinning and drawing, as well as punching, cutting, drilling and other machining operations. Also these methods include brazing, welding and soldering. There are achieved a wide variety of articles, products and component parts which then are readily heat-hardened by double heat-treatment, that is, a preliminary hardening treatment followed by a final hardening treatment. The finally hardened steel is hard and strong at room temperatures and at elevated temperatures as well. Moreover, it possesses good ductility and toughness. The strength and toughness of my steel lies not only in the direction of rolling or other working but also in the transverse directions of width and thickness. The steel has good corrosion resistance, particularly resisting intergranular corrosion.

Since many possible embodiments may be made of my invention and since many changes made in the embodiments herein set forth, it is to be understood that all matter described herein is to be interpreted as illustrative, and not as a limitation.

I claim as my invention:

1. A chromium-nickel-aluminum stainless steel susceptible to precipitation-hardening by double heat-treatment from a soft, workable, austenitic condition to give great strength in combination with good ductility, said steel consisting essentially of 9.00% to 20.00% chromium, 2.50% to 8.00% nickel, .70% to 2.50% aluminum, 1% to 5% molybdenum, with the sum of the chromium and molybdenum contents 14% to 21%, .10% to .40% nitrogen, car-

bon .12% maximum, manganese 8.00% maximum, with manganese inversely proportioned with respect to the nickel content, silicon 2.00% maximum, phosphorus .050% maximum, sulphur .050% maximum, and remainder substantially all iron.

2. A chromium-nickel-aluminum stainless steel susceptible to precipitation-hardening by double heat-treatment from a soft, workable, austenitic condition to give great strength in combination with good ductility, said steel consisting essentially of 15.0% to 16.0% chromium, 6.0% to 7.5% nickel, .8% to 1.5% aluminum, 2.0% to 3.0% molybdenum, .10% to .20% nitrogen, carbon .08% maximum, manganese 2% maximum, silicon 1.00% maximum, phosphorus .050% maximum, sulphur .050% maximum, and remainder substantially all iron.

3. A chromium-nickel-aluminum stainless steel susceptible to precipitation-hardening by double heat-treatment from a soft, workable, austenitic condition to give great strength in combination with good ductility, said steel consisting essentially of 15.0% to 16.0% chromium, 6.0% to 7.5% nickel, .8% to 1.5% aluminum, 2.0% to 3.0% molybdenum, .12% to .15% nitrogen, carbon .03% maxi-

mum, manganese 2% maximum, silicon 1.00% maximum, phosphorus .050% maximum, sulphur .050% maximum, balance iron.

4. A chromium-nickel-aluminum stainless steel precipitation-hardened by double heat-treatment from the annealed condition to give great strength in combination with good ductility and consisting essentially of 9% to 20% chromium, 2.50% to 8.00% nickel, .70% to 2.50% aluminum, 1% to 5% molybdenum, with the sum of the chromium and molybdenum contents 14% to 21%, .10% to .40% nitrogen, carbon .12% maximum, manganese 8.00% maximum, with manganese inversely proportioned to nickel and 8.00% when nickel is 2.5% and 2% maximum when nickel is 8.00%, silicon 2.00% maximum, phosphorus .050% maximum, sulphur .050% maximum, and remainder substantially all iron.

5. A chromium-nickel-aluminum stainless steel precipitation-hardened by double heat-treatment from the annealed condition to give a hardness of at least Rockwell C46, an ultimate strength of at least 200,000 p.s.i. all in combination with elongation in 2" of at least 12%, said steel consisting essentially of 15.0% to 16.5% chromium, 6.0% to 7.5% nickel, .8% to 1.5% aluminum, 2.0% to 3.0% molybdenum, .10% to .20% nitrogen, carbon .03% maximum, and remainder substantially all iron.

#### References Cited by the Examiner

#### UNITED STATES PATENTS

|           |         |                      |          |
|-----------|---------|----------------------|----------|
| 1,831,946 | 11/1931 | Breeler -----        | 75—124   |
| 2,223,659 | 12/1940 | Harders et al. ----- | 75—128.5 |
| 2,505,763 | 5/1950  | Goller -----         | 75—124   |
| 2,868,637 | 1/1959  | Kirkpatrick -----    | 75—124   |
| 2,892,702 | 6/1959  | Walton et al. -----  | 75—124   |

DAVID L. RECK, Primary Examiner.

RAY K. WINDHAM, MARCUS U. LYONS, Examiners.